



US006426038B1

(12) **United States Patent**  
**Fedchun**

(10) **Patent No.:** **US 6,426,038 B1**  
(45) **Date of Patent:** **Jul. 30, 2002**

(54) **UNIVERSAL ALLOY STEEL**

(75) Inventor: **Vladimir A. Fedchun**, Farmington Hills, MI (US)

(73) Assignee: **Modern Alloy Co., LLC**, Farmington Hills, MI (US)

(\*) Notice: Subject to any disclaimer, the term of this patent is extended or adjusted under 35 U.S.C. 154(b) by 0 days.

(21) Appl. No.: **09/534,117**

(22) Filed: **Mar. 23, 2000**

**Related U.S. Application Data**

(60) Division of application No. 09/003,923, filed on Jan. 7, 1998, now Pat. No. 6,187,261, which is a continuation-in-part of application No. PCT/RU96/00184, filed on Jul. 9, 1996, and a continuation-in-part of application No. PCT/RU96/00230, filed on Aug. 15, 1996.

(51) **Int. Cl.<sup>7</sup>** ..... **C22C 38/02**

(52) **U.S. Cl.** ..... **420/34**; 420/60; 420/90; 420/104

(58) **Field of Search** ..... 420/8, 34, 60, 420/90, 104, 127

(56) **References Cited**

**U.S. PATENT DOCUMENTS**

4,650,645 A \* 3/1987 Kato et al. .... 420/111  
5,055,253 A \* 10/1991 Nelson .... 420/87  
5,616,187 A \* 4/1997 Nelson .... 148/333  
5,928,442 A \* 7/1999 Machmeier et al. .... 148/335

\* cited by examiner

*Primary Examiner*—Ngoclan Mai

(57) **ABSTRACT**

A composition and method for reducing cost and improving the mechanical properties of alloy steels. The invention resides in the ability of certain combinations of carbon-subgroup surfactants and d-transition metals to modify and control diffusion mechanisms of interstitial elements; to reduce or prevent the formation of non-equilibrium segregations of harmful admixtures and brittle phases on free metal surfaces and grain and phase boundaries; and to alter and control phase transformation kinetics in steel during heating and cooling.

**3 Claims, 13 Drawing Sheets**

## Classification of Universal Steels

| Type                       | Class | Classification                    | Alloying System | Figure |
|----------------------------|-------|-----------------------------------|-----------------|--------|
| General Engineering Steels | I     | High Ductility Steel              | 10CrABC         | 2      |
|                            | II    | Case Hardening Steel              | 25CrABC         | 3      |
|                            | III   | Direct Hardening, Nitriding Steel | 40CrABC         | 4 5 6  |
|                            | IV    | Direct Hardening, Nitriding Steel | 50CrABC         | 7      |
|                            | V     | Tool Steel                        | 60CrABC         | 8      |
|                            | VI    | Maraging Steel                    | 10Cr10Ni8ABC    | 13     |
|                            | VII   | High Ductility Steel              | 10Cr16ABC       | 9      |
|                            | VIII  | Direct Hardening Steel            | 40Cr16ABC       | 10 11  |
|                            | IX    | Tool Steel                        | 60Cr16ABC       | 12     |
| Stainless Steels           |       |                                   |                 |        |

Figure 1

**General Engineering Universal Steel**  
**High Ductility Steel**

| Alloying System                           | (Si+Cu)/V | Chemical Composition, wt. % |                                          |            |               |                   |                                       |        |       |
|-------------------------------------------|-----------|-----------------------------|------------------------------------------|------------|---------------|-------------------|---------------------------------------|--------|-------|
|                                           |           | C                           | Mn                                       | Si         | Cr            | Cu                | V                                     | S      | P     |
| <b>Heat Treatment</b>                     |           |                             |                                          |            |               |                   |                                       |        |       |
| Si - Cu - V                               | 8.23      | 0.10                        | 0.47                                     | 0.84       | 0.62          | 0.56              | 0.17                                  | 0.025  | 0.021 |
| Due to Mill Rolling Only                  | 260       | 680                         | 490                                      | 24         | 70            | 70                | 200                                   | 182    | 180   |
| <b>Static and Dynamic Characteristics</b> |           |                             |                                          |            |               |                   |                                       |        |       |
|                                           |           | Brinell Hardness            | Tensile Min. Strength, N/mm <sup>2</sup> | Est. Yield | Elongation, % | Reduction Area, % | <b>Impact Value, J/cm<sup>2</sup></b> |        |       |
|                                           |           |                             |                                          |            |               |                   | KCU                                   | KCV    |       |
|                                           |           |                             |                                          |            |               |                   | + 20°C                                | - 60°C |       |
|                                           |           |                             |                                          |            |               |                   |                                       |        |       |
| <b>Heat Treatment</b>                     |           |                             |                                          |            |               |                   |                                       |        |       |
| Ge - Cu - V                               | 6.72      | 0.12                        | 0.51                                     | 0.17       | 0.57          | 0.74              | 0.47                                  | 0.18   | 0.025 |
| Due to Mill Rolling Only                  | 245       | 650                         | 570                                      | 26         | 76            | 76                | 220                                   | 200    | 190   |
| <b>Static and Dynamic Characteristics</b> |           |                             |                                          |            |               |                   |                                       |        |       |
|                                           |           | Brinell Hardness            | Tensile Min. Strength, N/mm <sup>2</sup> | Est. Yield | Elongation, % | Reduction Area, % | <b>Impact Value, J/cm<sup>2</sup></b> |        |       |
|                                           |           |                             |                                          |            |               |                   | KCU                                   | KCV    |       |
|                                           |           |                             |                                          |            |               |                   | + 20°C                                | - 60°C |       |
|                                           |           |                             |                                          |            |               |                   |                                       |        |       |

Figure 2

**General Engineering Universal Steel**  
**Case Hardening Steel**

| Alloying System                    | $(\text{Si}+\text{Cu})/\text{V}$ | Chemical Composition, wt. %              |            |               |                   |                                 |      |       |        |
|------------------------------------|----------------------------------|------------------------------------------|------------|---------------|-------------------|---------------------------------|------|-------|--------|
|                                    |                                  | C                                        | Mn         | Si            | Cr                | Cu                              | V    | S     | P      |
| Si - Cu - V                        | 6.81                             | 0.27                                     | 0.38       | 0.92          | 0.74              | 0.58                            | 0.22 | 0.019 | 0.02   |
| Heat Treatment                     | Rockwell Hardness                | Tensile Min. Strength, N/mm <sup>2</sup> | Est. Yield | Elongation, % | Reduction Area, % | Impact Value, J/cm <sup>2</sup> |      |       |        |
| Static and Dynamic Characteristics |                                  |                                          |            |               |                   |                                 |      |       |        |
| Quenching, Low Temper.             | C38                              | 1256                                     | 998        | 15            | 49                | + 20°C                          | KCU  | KCV   | - 40°C |
| Carburizing, Quench, Low Tempering | C56                              | 1690                                     | 1615       | 8.1           | 26.4              | 68                              | 43   | 29    | 22     |
|                                    |                                  |                                          |            |               |                   | 24                              | 16   | 12.2  | 9.8    |

  

| Alloying System                    | $(\text{Ge}+\text{Cu})/\text{V}$ | Chemical Composition, wt. %              |            |               |                   |                                 |      |      |        |      |
|------------------------------------|----------------------------------|------------------------------------------|------------|---------------|-------------------|---------------------------------|------|------|--------|------|
|                                    |                                  | C                                        | Mn         | Si            | Cr                | Ge                              | Cu   | V    | S      | P    |
| Ge - Cu - V                        | 6.34                             | 0.25                                     | 0.42       | 0.18          | 0.64              | 0.92                            | 0.54 | 0.23 | 0.02   | 0.02 |
| Heat Treatment                     | Rockwell Hardness                | Tensile Min. Strength, N/mm <sup>2</sup> | Est. Yield | Elongation, % | Reduction Area, % | Impact Value, J/cm <sup>2</sup> |      |      |        |      |
| Static and Dynamic Characteristics |                                  |                                          |            |               |                   |                                 |      |      |        |      |
| Quenching, Low Tempering           | C36                              | 1220                                     | 1150       | 17            | 51                | + 20°C                          | KCU  | KCV  | - 40°C |      |
| Carburizing, Quench, Low Tempering | C56                              | 1720                                     | 1670       | 10.4          | 32                | 74                              | 51   | 32   | 25     |      |
|                                    |                                  |                                          |            |               |                   | 36                              | 21   | 16.2 | 11.6   |      |

Figure 3

**General Engineering Universal Steel  
Direct Hardening, Nitriding Steel**

| Alloying System | (Si+Cu)/V            | Chemical Composition, wt. %        |                                          |            |               |                   |                                 |                                 |  |
|-----------------|----------------------|------------------------------------|------------------------------------------|------------|---------------|-------------------|---------------------------------|---------------------------------|--|
|                 |                      | C                                  | Mn                                       | Si         | Cr            | Cu                | V                               | S                               |  |
|                 | 6.08                 | 0.39                               | 0.27                                     | 0.87       | 1.99          | 0.59              | 0.24                            | 0.021                           |  |
| Heat            |                      | Static and Dynamic Characteristics |                                          |            |               |                   |                                 | Impact Value, J/cm <sup>2</sup> |  |
|                 | Treatment            | Rockwell Hardness                  | Tensile Min. Strength, N/mm <sup>2</sup> | Est. Yield | Elongation, % | Reduction Area, % | Impact Value, J/cm <sup>2</sup> |                                 |  |
| Si - Cu - V     | Quenching at 890°C   | C55                                | 2010                                     | 1890       | 10            | 42                | + 20°C                          |                                 |  |
|                 | Low Temper at 200°C  | C46                                | 1510                                     | 1470       | 13            | 45                | 64                              | 42                              |  |
|                 | Quenching at 890°C   | C28                                | 910                                      | 874        | 23            | 65                | 59                              | 40                              |  |
|                 | Mid. Temper at 500°C |                                    |                                          |            |               |                   | 36                              | 34                              |  |
|                 | Quenching at 890°C   |                                    |                                          |            |               |                   | 76                              | 76                              |  |
|                 | High Temper at 650°C |                                    |                                          |            |               |                   | 67                              | 67                              |  |

**Figure 4**

**General Engineering Universal Steel**  
**Direct Hardening, Nitriding Steel**

| Alloying System | $(\text{Ge}+\text{Cu})/\text{V}$        | Chemical Composition, wt. %              |            |               |                   |                                 |        | P   |
|-----------------|-----------------------------------------|------------------------------------------|------------|---------------|-------------------|---------------------------------|--------|-----|
|                 |                                         | C                                        | Mn         | Si            | Cr                | Ge                              | Cu     |     |
| Heat Treatment  | Rockwell Hardness                       | Tensile Min. Strength, N/mm <sup>2</sup> | Est. Yield | Elongation, % | Reduction Area, % | Impact Value, J/cm <sup>2</sup> |        |     |
| Ge - Cu - V     | Quenching at 890°C Low Temper at 200°C  | C56                                      | 2180       | 1970          | 12                | 48                              | + 20°C |     |
|                 | Quenching at 890°C Mid. Temper at 500°C | C47                                      | 1615       | 1590          | 14                | 52                              | 78     | 59  |
|                 | Quenching at 890°C High Temper at 650°C | C29                                      | 1050       | 990           | 25                | 68                              | 180    | 120 |
|                 |                                         |                                          |            |               |                   |                                 | 98     | 98  |
|                 |                                         |                                          |            |               |                   |                                 | 46     | 84  |

**Figure 5**

**General Engineering Universal Steel**  
**Direct Hardening Steel, Nitriding Steel**

| Alloying System                           | (Si+Cu)/V              | Chemical Composition, wt. %                         |                          |                                     |                                               |                                             |                   | P    |
|-------------------------------------------|------------------------|-----------------------------------------------------|--------------------------|-------------------------------------|-----------------------------------------------|---------------------------------------------|-------------------|------|
|                                           |                        | C                                                   | Mn                       | Si                                  | Cr                                            | Cu                                          | V                 |      |
| <b>Service Operations Characteristics</b> |                        |                                                     |                          |                                     |                                               |                                             |                   |      |
| Treatment                                 | Core Hardness Rockwell | Nitrided Layer Surf. Hardness HV, N/mm <sup>2</sup> | Nitrided Layer Depth, mm | Impact Value, KCU J/cm <sup>2</sup> | Ultimate Contact Endurance, N/mm <sup>2</sup> | Ultimate Fatigue Strength N/mm <sup>2</sup> | Wear Resistance * |      |
| Si - Cu - V                               |                        |                                                     |                          |                                     |                                               |                                             |                   |      |
| Ion Nitriding 500°C, 24 hrs.              | C45                    | 8400                                                | 0.64                     | 52                                  | 2200                                          | 620                                         | 1.24              |      |
| <b>Chemical Composition, wt. %</b>        |                        |                                                     |                          |                                     |                                               |                                             |                   |      |
| Alloying System                           | (Ge+Cu)/V              | C                                                   | Mn                       | Si                                  | Cr                                            | Ge                                          | Cu                | V    |
| Ge - Cu - V                               | 9.35                   | 0.41                                                | 0.44                     | 0.18                                | 1.87                                          | 0.97                                        | 0.62              | 0.17 |
|                                           |                        |                                                     |                          |                                     |                                               |                                             |                   |      |
|                                           |                        |                                                     |                          |                                     |                                               |                                             |                   |      |
|                                           |                        |                                                     |                          |                                     |                                               |                                             |                   |      |
|                                           |                        |                                                     |                          |                                     |                                               |                                             |                   |      |
| <b>Static and Dynamic Characteristics</b> |                        |                                                     |                          |                                     |                                               |                                             |                   |      |
| Treatment                                 | Core Hardness Rockwell | Nitrided Layer Surf. Hardness HV, N/mm <sup>2</sup> | Nitrided Layer Depth, mm | Impact Value, KCU J/cm <sup>2</sup> | Ultimate Contact Endurance, N/mm <sup>2</sup> | Ultimate Fatigue Strength N/mm <sup>2</sup> | Wear Resistance * |      |
| Ion Nitriding 500°C, 24 hrs.              | C42                    | 7900                                                | 0.78                     | 65                                  | 2350                                          | 740                                         | 1.42              |      |

\* wear resistance of bearing steel 1MX15Cr, heat treated to HRC 62 is assumed to be equal to 1.

**Figure 6**

**General Engineering Universal Steel**  
**Direct Hardening, Nitriding Steel**

| Alloying System                            | (Si+Cu)V                                   | Chemical Composition, wt. %              |            |               |                   |                                    |                                    |        |      |    |  |  |  |
|--------------------------------------------|--------------------------------------------|------------------------------------------|------------|---------------|-------------------|------------------------------------|------------------------------------|--------|------|----|--|--|--|
|                                            |                                            | C                                        | Mn         | Si            | Cr                | Cu                                 | V                                  | S      | P    |    |  |  |  |
| Si - Cu - V                                | 6.66                                       | 0.54                                     | 0.78       | 1.02          | 0.86              | 0.58                               | 0.24                               | 0.021  | 0.02 |    |  |  |  |
|                                            | Quenching at 890°C<br>Low Temper at 180°C  | C56                                      | 2310       | 1990          | 8                 | 27                                 | Static and Dynamic Characteristics |        |      |    |  |  |  |
| Alloying System                            | (Ge+Cu)V                                   | Chemical Composition, wt. %              |            |               |                   |                                    |                                    |        |      |    |  |  |  |
|                                            |                                            | C                                        | Mn         | Si            | Cr                | Ge                                 | Cu                                 | V      | S    | P  |  |  |  |
| Heat Treatment                             | Rockwell Hardness                          | Tensile Min. Strength, N/mm <sup>2</sup> | Est. Yield | Elongation, % | Reduction Area, % | Static and Dynamic Characteristics |                                    |        |      |    |  |  |  |
|                                            | Quenching at 890°C<br>Mid.Temper at 380°C  | C52                                      | 1920       | 1895          | 8.5               | 29                                 | Impact Value, J/cm <sup>2</sup>    |        |      |    |  |  |  |
| Ge - Cu - V                                |                                            |                                          |            |               |                   |                                    | + 20°C                             | - 60°C |      |    |  |  |  |
| Quenching at 890°C<br>Mid.Temper at 380°C  |                                            |                                          |            |               |                   |                                    | 36                                 | 23     | 21   | 16 |  |  |  |
| Alloying System                            | (Ge+Cu)V                                   | Chemical Composition, wt. %              |            |               |                   |                                    |                                    |        |      |    |  |  |  |
|                                            |                                            | C                                        | Mn         | Si            | Cr                | Ge                                 | Cu                                 | V      | S    | P  |  |  |  |
| Heat Treatment                             | Rockwell Hardness                          | Tensile Min. Strength, N/mm <sup>2</sup> | Est. Yield | Elongation, % | Reduction Area, % | Static and Dynamic Characteristics |                                    |        |      |    |  |  |  |
|                                            | Quenching at 890°C<br>Low Temper. at 180°C | C54                                      | 2230       | 2190          | 12                | 35                                 | Impact Value, J/cm <sup>2</sup>    |        |      |    |  |  |  |
| Alloying System                            |                                            |                                          |            |               |                   |                                    | + 20°C                             | - 60°C |      |    |  |  |  |
| Quenching at 890°C<br>Mid.Temper. at 380°C |                                            |                                          |            |               |                   |                                    | 48                                 | 36     | 34   | 27 |  |  |  |
| Alloying System                            | (Ge+Cu)V                                   | Chemical Composition, wt. %              |            |               |                   |                                    |                                    |        |      |    |  |  |  |
|                                            |                                            | C                                        | Mn         | Si            | Cr                | Ge                                 | Cu                                 | V      | S    | P  |  |  |  |
| Heat Treatment                             | Rockwell Hardness                          | Tensile Min. Strength, N/mm <sup>2</sup> | Est. Yield | Elongation, % | Reduction Area, % | Static and Dynamic Characteristics |                                    |        |      |    |  |  |  |
|                                            | Quenching at 890°C<br>Mid.Temper. at 380°C | C50                                      | 1860       | 1810          | 13                | 40                                 | Impact Value, J/cm <sup>2</sup>    |        |      |    |  |  |  |
| Alloying System                            | (Ge+Cu)V                                   | Chemical Composition, wt. %              |            |               |                   |                                    |                                    |        |      |    |  |  |  |
|                                            |                                            | C                                        | Mn         | Si            | Cr                | Ge                                 | Cu                                 | V      | S    | P  |  |  |  |
| Heat Treatment                             | Rockwell Hardness                          | Tensile Min. Strength, N/mm <sup>2</sup> | Est. Yield | Elongation, % | Reduction Area, % | Static and Dynamic Characteristics |                                    |        |      |    |  |  |  |
|                                            | Quenching at 890°C<br>Mid.Temper. at 380°C | C50                                      | 1860       | 1810          | 13                | 40                                 | Impact Value, J/cm <sup>2</sup>    |        |      |    |  |  |  |

Figure 7

**General Engineering Universal Steel  
Tool Steel**

| Alloying System     | (Si+Cu)/V      | Chemical Composition, wt. % |                                          |            |               |                   |                                 | P     |
|---------------------|----------------|-----------------------------|------------------------------------------|------------|---------------|-------------------|---------------------------------|-------|
|                     |                | C                           | Mn                                       | Si         | Cr            | Cu                | V                               |       |
| Si - Cu - V         | 6.12           | 0.63                        | 0.81                                     | 0.97       | 1.14          | 0.56              | 0.25                            | 0.023 |
|                     | Heat Treatment | Brinell Hardness            | Tensile Min. Strength, N/mm <sup>2</sup> | Est. Yield | Elongation, % | Reduction Area, % | Impact Value, J/cm <sup>2</sup> |       |
| Quenching at 860°C  | C62            | 2450                        | 2290                                     | 6          | 24            | + 20°C            | KCU                             | KCV   |
| Low Temper at 180°C |                |                             |                                          |            |               | - 40°C            | KCU                             | KCV   |

  

| Alloying System     | (Ge+Cu)/V        | Chemical Composition, wt. %              |            |               |                      |                                 |      | P     |
|---------------------|------------------|------------------------------------------|------------|---------------|----------------------|---------------------------------|------|-------|
|                     |                  | C                                        | Mn         | Si            | Cr                   | Ge                              | Cu   |       |
| Ge - Cu - V         | 5.4              | 0.58                                     | 0.74       | 0.32          | 1.27                 | 0.98                            | 0.48 | 0.022 |
| Heat Treatment      | Brinell Hardness | Tensile Min. Strength, N/mm <sup>2</sup> | Est. Yield | Elongation, % | Reduction in Area, % | Impact Value, J/cm <sup>2</sup> |      |       |
| Quenching at 860°C  | C60              | 2410                                     | 2370       | 8             | 32                   | + 20°C                          | KCU  | KCV   |
| Low Temper at 180°C |                  |                                          |            |               |                      | - 40°C                          |      |       |

Figure 8

**Stainless Universal Steel  
High Ductility Steel**

| Alloying System       | $(\text{Si}+\text{Cu})/\text{V}$ | Chemical Composition, wt. % |      |      |      |      |      |       |       |
|-----------------------|----------------------------------|-----------------------------|------|------|------|------|------|-------|-------|
|                       |                                  | C                           | Mn   | Si   | Cr   | Cu   | V    | S     | P     |
| <b>Heat Treatment</b> |                                  |                             |      |      |      |      |      |       |       |
| Si - Cu - V           | 6.77                             | 0.12                        | 0.18 | 0.85 | 16.2 | 0.64 | 0.22 | 0.021 | 0.019 |
| Rolling               | 240                              | 670                         | 520  |      | 22   |      | 60   |       | 82    |
| High Tempering        |                                  |                             |      |      |      |      |      |       |       |

| Alloying System       | $(\text{Ge}+\text{Cu})/\text{V}$ | Chemical Composition, wt. % |      |      |      |      |      |      |      |       |
|-----------------------|----------------------------------|-----------------------------|------|------|------|------|------|------|------|-------|
|                       |                                  | C                           | Mn   | Si   | Cr   | Ge   | Cu   | V    | S    | P     |
| <b>Heat Treatment</b> |                                  |                             |      |      |      |      |      |      |      |       |
| Ge - Cu - V           | 5.91                             | 0.15                        | 0.21 | 0.14 | 15.8 | 0.88 | 0.54 | 0.24 | 0.02 | 0.021 |
| Rolling               | 260                              | 680                         | 560  |      | 24   |      | 65   |      | 98   |       |
| High Tempering        |                                  |                             |      |      |      |      |      |      |      |       |

Figure 9

**Stainless Universal Steel  
Direct Hardening Steel**

| Alloying System                           | $(\text{Si}+\text{Cu})/\text{V}$ | Chemical Composition, wt. % |                                          |            |               |                      |                                      |       |       |       |
|-------------------------------------------|----------------------------------|-----------------------------|------------------------------------------|------------|---------------|----------------------|--------------------------------------|-------|-------|-------|
|                                           |                                  | C                           | Mn                                       | Si         | Cr            | Cu                   | V                                    | S     |       |       |
| <b>Static and Dynamic Characteristics</b> |                                  |                             |                                          |            |               |                      |                                      |       |       |       |
| Si - Cu - V                               |                                  | Rockwell Hardness           | Tensile Min. Strength, N/mm <sup>2</sup> | Est. Yield | Elongation, % | Reduction Area, %    | Impact Value, KCU, J/cm <sup>2</sup> |       |       |       |
| Quenching at 1100°C                       | 14.4                             | 0.45                        | 0.27                                     | 1.01       | 16.7          | 0.72                 | 0.12                                 | 0.021 |       |       |
|                                           | Low Tempering at 200°C           | C59                         | 2115                                     | 1920       | 6             | 15                   | 36                                   | 0.019 |       |       |
| Alloying System                           | $(\text{Ge}+\text{Cu})/\text{V}$ | Chemical Composition, wt. % |                                          |            |               |                      |                                      |       |       |       |
|                                           |                                  | C                           | Mn                                       | Si         | Cr            | Ge                   | Cu                                   | V     | S     | P     |
| <b>Static and Dynamic Characteristics</b> |                                  |                             |                                          |            |               |                      |                                      |       |       |       |
| Ge - Cu - V                               | 8.83                             | 0.42                        | 0.24                                     | 0.17       | 15.9          | 0.98                 | 0.61                                 | 0.18  | 0.019 | 0.019 |
| Quenching at 1100°C                       | Heat Treatment                   | Rockwell Hardness           | Tensile Min. Strength, N/mm <sup>2</sup> | Est. Yield | Elongation, % | Reduction in Area, % | Impact Value, KCU, J/cm <sup>2</sup> |       |       |       |
|                                           | Low Tempering at 200°C           | C56                         | 2020                                     | 1890       | 8             | 22                   | 54                                   |       |       |       |

**Figure 10**

## Stainless Universal Steel, Direct Hardening Steel

| Alloying System           | (Si+Cu)/V                                   | Chemical Composition, wt. %   |                                      |     |              |                            |   | P |
|---------------------------|---------------------------------------------|-------------------------------|--------------------------------------|-----|--------------|----------------------------|---|---|
|                           |                                             | C                             | Mn                                   | Si  | Cr           | Cu                         | V |   |
| Heat Treatment            | Agent and Test Conditions                   |                               | Corrosion Resistance Characteristics |     | Durability * |                            |   |   |
| (Si +Cu)/V                | H <sub>2</sub> SO <sub>4</sub> (93%), +20°C |                               |                                      | 288 |              | 3 durable enough           |   |   |
|                           | Quenching at 1100°C                         |                               |                                      | 600 |              | 4 durable under activation |   |   |
|                           | Low Tempering at 200°C                      | HNO <sub>3</sub> (56%), +20°C |                                      | 288 |              | 4 durable                  |   |   |
|                           | Sea Water + 400 ml. H <sub>2</sub> S, +20°C |                               |                                      | 600 |              | 1 absolutely durable       |   |   |
|                           | Na Cl (3%), at boiling t°C                  |                               |                                      | 790 |              | 2 durable enough           |   |   |
| (Ge +Cu)/V                | Na Cl (3%), at boiling t°C                  |                               |                                      | 60  |              | 4 durable                  |   |   |
| Alloying System           | (Ge+Cu)/V                                   | Chemical Composition, wt. %   |                                      |     |              |                            |   | P |
| Heat Treatment            | Agent and Test Conditions                   |                               | Corrosion Resistance Characteristics |     | Durability * |                            |   |   |
| (Ge +Cu)/V                | H <sub>2</sub> SO <sub>4</sub> (93%), +20°C |                               |                                      | 288 |              | 2 durable enough           |   |   |
|                           | Quenching at 1100°C                         |                               |                                      | 600 |              | 2 durable under activation |   |   |
|                           | Low Tempering at 200°C                      | HNO <sub>3</sub> (56%), +20°C |                                      | 288 |              | 3 durable                  |   |   |
|                           | Sea Water + 400 ml. H <sub>2</sub> S, +20°C |                               |                                      | 600 |              | 1 absolutely durable       |   |   |
|                           | Na Cl (3%), at boiling t°C                  |                               |                                      | 790 |              | 1 durable enough           |   |   |
| * Index per GOST 13619-68 |                                             |                               |                                      |     |              |                            |   |   |

Figure 11

**Stainless Universal Steel  
Tool Steel**

| Alloying System                           | $(\text{Si}+\text{Cu})/\text{V}$ | Chemical Composition, wt. %                    |                   |                      |                          |                                           |      | P     |
|-------------------------------------------|----------------------------------|------------------------------------------------|-------------------|----------------------|--------------------------|-------------------------------------------|------|-------|
|                                           |                                  | C                                              | Mn                | Si                   | Cr                       | Cu                                        | V    |       |
|                                           | 10.4                             | 0.63                                           | 0.17              | 0.84                 | 16.2                     | 0.72                                      | 0.15 | 0.023 |
| <b>Static and Dynamic Characteristics</b> |                                  |                                                |                   |                      |                          |                                           |      |       |
| <b>Heat Treatment</b>                     | <b>Rockwell Hardness</b>         | <b>Tensile Min. Strength, N/mm<sup>2</sup></b> | <b>Est. Yield</b> | <b>Elongation, %</b> | <b>Reduction Area, %</b> | <b>Impact Value, KCU J/cm<sup>2</sup></b> |      |       |
| Si - Cu - V                               | Quenching at 1100°C              | C61                                            | 2180              | 1750                 | 3                        | 11                                        | 25   |       |
|                                           | Low Tempering at 200°C           |                                                |                   |                      |                          |                                           |      |       |

  

| Alloying System                           | $(\text{Ge}+\text{Cu})/\text{V}$ | Chemical Composition, wt. %                    |                   |                      |                          |                                           |      | P     |
|-------------------------------------------|----------------------------------|------------------------------------------------|-------------------|----------------------|--------------------------|-------------------------------------------|------|-------|
|                                           |                                  | C                                              | Mn                | Si                   | Cr                       | Ge                                        | Cu   |       |
|                                           | 6.63                             | 0.60                                           | 0.21              | 0.18                 | 16.8                     | 1.02                                      | 0.44 | 0.020 |
| <b>Static and Dynamic Characteristics</b> |                                  |                                                |                   |                      |                          |                                           |      |       |
| <b>Heat Treatment</b>                     | <b>Rockwell Hardness</b>         | <b>Tensile Min. Strength, N/mm<sup>2</sup></b> | <b>Est. Yield</b> | <b>Elongation, %</b> | <b>Reduction Area, %</b> | <b>Impact Value, KCU J/cm<sup>2</sup></b> |      |       |
| Ge - Cu - V                               | Quenching at 1100°C              | C59                                            | 2150              | 1910                 | 7                        | 18                                        | 42   |       |
|                                           | Low Tempering at 200°C           |                                                |                   |                      |                          |                                           |      |       |

Figure 12

**General Engineering Universal Steel  
Maraging Steel**

| Alloying System                           | (Si+Cu)/V                                  | Chemical Composition, wt. %              |            |               |                   |                                     |              |              |              |
|-------------------------------------------|--------------------------------------------|------------------------------------------|------------|---------------|-------------------|-------------------------------------|--------------|--------------|--------------|
|                                           |                                            | C                                        | Ni         | Si            | Cr                | Cu                                  | V            | S            | P            |
|                                           | 2.35                                       | 0.10                                     | 8.4        | 0.92          | 11.2              | 0.64                                | 0.67         | 0.018        | 0.019        |
| <b>Static and Dynamic Characteristics</b> |                                            |                                          |            |               |                   |                                     |              |              |              |
| Heat Treatment                            | Rockwell Hardness                          | Tensile Min. Strength, N/mm <sup>2</sup> | Est. Yield | Elongation, % | Reduction Area, % | Impact Value, KCU J/cm <sup>2</sup> |              |              |              |
| Si - Cu - V                               | Quenching at 980°C<br>Mid. Temper at 450°C | C44                                      | 1350       | 1320          | 24                | 72                                  | +20°C<br>180 | -196°C<br>82 | -253°C<br>54 |

  

| Alloying System                           | (Ge+Cu)/V                                  | Chemical Composition, wt. %              |            |               |                   |                                     |              |               |              |
|-------------------------------------------|--------------------------------------------|------------------------------------------|------------|---------------|-------------------|-------------------------------------|--------------|---------------|--------------|
|                                           |                                            | C                                        | Ni         | Si            | Cr                | Ge                                  | Cu           | V             | S            |
| <b>Static and Dynamic Characteristics</b> |                                            |                                          |            |               |                   |                                     |              |               |              |
| Heat Treatment                            | Rockwell Hardness                          | Tensile Min. Strength, N/mm <sup>2</sup> | Est. Yield | Elongation, % | Reduction Area, % | Impact Value, KCU J/cm <sup>2</sup> |              |               |              |
| Ge - Cu - V                               | Quenching at 980°C<br>Mid. Temper at 450°C | C44                                      | 1340       | 1335          | 28                | 79                                  | +20°C<br>220 | -196°C<br>102 | -253°C<br>61 |

Figure 13

## UNIVERSAL ALLOY STEEL

## RELATED APPLICATIONS

This is a divisional application of a copending application Ser. No. 09/003,923 filed on Jan. 7, 1998 U.S. Pat. No. 6,187,261, which is a continuation-in-part of PCT patent application Ser. No. PCT/RU96/00184 filed on Jul. 9, 1996, and PCT patent application Ser. No. PCT/RU96/00230 filed on Aug. 15, 1996.

## FIELD OF THE INVENTION

This invention relates to steel alloys, commonly designated as specialty steels, and more particularly to steel alloy systems and methods for improving the mechanical properties of alloy steels, reducing the complexity of alloy steel compositions and reducing costs.

## BACKGROUND OF THE INVENTION

The mechanical properties of alloy steels vary with the properties of their free metal boundaries, grain bodies and grain and phase boundaries. Current practices rely on many alloying systems and thermomechanical treatments, such as rolling, pressing, hammering and forging and various chemical and heat treatments to alter the mechanical properties of alloy steels. Current alloying systems are based on the idea of steel microstructure modifications and do not consider the effects of grain boundaries between crystals and alloy phase components on mechanical properties.

Iron (Fe), carbon (C), manganese (Mn), phosphorus (P), sulfur (S), silicon (Si), and traces of oxygen (O), nitrogen (N), and aluminum (Al) are always present in steel, together with alloying elements, such as nickel (Ni), chromium (Cr), copper (Cu), molybdenum (Mo), tungsten (W), cobalt (Co) and vanadium (V). Current alloying systems, steel making and heat treatment practices often procure non-equilibrium segregations of traditionally harmful admixtures (S, P, Sn, etc.), as well as embrittling non-metallic phases on free metal surfaces, grain and phase boundaries during tempering. Chemical heat treatments, such as nitro-carburizing and nitriding cause brittleness and distortion of grain bodies due to formation of a second, large volume phase along grain boundaries, having a harmful effect on the viscous characteristics of steel. For example, the impact strength of steel containing (by weight) 0.25% C; 1.6% Cr; 1.5% Ni; 1.0% W; and 0.6% Mo, is reduced to 2-3 J/cm<sup>2</sup>, following oil quenching at 980° C. and a 24 hour tempering at 500° C. (so-called false nitriding).

Another aspect of current steel alloying, making and heat treatment practices is that increases in strength decrease ductility, and in the alternative, increases in ductility decrease strength. Heretofore, no satisfactory compromise has been found between strength and ductility of alloy steels.

Current practices require large numbers of classes and grades of alloy steels, large investments and large inventories to support the requirements of industrial and consumer products. More than 320 grades of specialty steels are produced in the United States; 70-100 in Germany; 140-160 in Great Britain; 60-70 in Sweden; 140-160 in France; 100-120 in Japan; and 140-150 in Russia.

The following alloying systems are typical of current practices:

A: Structural, heat-treatable, carburizing, nitro-carburizing, and nitriding steels 1.

1. Fe—C—Cr
2. Fe—C—Cr—Mo—Al
3. Fe—C—Cr—Ni—Mo

## B. Die, spring, maraging, and duplex steels

1. Fe—C—Cr—Si
2. Fe—C—Cr—Si—V—B
3. Fe—C—Cr—Si—Ni—Mo—(V, Ti)—N
- C. High speed tool steels
1. Fe—C—Cr—W—Mo—V—Co.
- D. High temperature steels
1. Fe—C—Cr—Ni—Mo—Si—(V, Ti, Nb)
- E. Free-cutting steels
1. Fe—C—Cr—(Ca, Pb, Se, Te, Sb)

Another aspect of the current practice is that vast, complex facilities are required to support the many current alloying systems. Large sums of money are required to establish and maintain large inventories and complex facilities.

## SUMMARY OF THE INVENTION

One benefit of the present invention is that strength of steels can be increased without significant reductions in ductility, or in the alternative, ductility can be increased without significant reductions in strength. Another major benefit is that the number of grades of specialty steels for meeting industrial and consumer requirements can be substantially reduced. Still another benefit is that number and complexity of steel making facilities can be substantially reduced. Yet another benefit is that substantial savings can be made in reducing inventories. One more benefit is that various grades of steel can be produced by using a continuous-casting furnace, varying the amount of carbon during melting; better commonality can be achieved for all subsequent metallurgical conversion processes (casting, heating, rolling, heat treatment). Still yet another benefit is that the use of expensive alloying elements, such as nickel (Ni), molybdenum (Mo), titanium (Ti), cobalt (Co), boron (B), and tungsten (W) can be eliminated, except for maraging steels.

The invention resides in the ability of certain combinations of carbon-subgroup surfactants and d-transition metals, which will be described in proper sequence, in  $\alpha$  and  $(\alpha+\gamma)$  steels to: 1) modify and control diffusion mechanisms of interstitial elements; 2) reduce or prevent the formation of non-equilibrium segregations of harmful admixtures and brittle phases being formed on free metal surfaces, grain and phase boundaries; 3) alter and control the phase transformation kinetics in steel during heating and cooling.

In a first embodiment of the invention, combinations of silicon, copper and vanadium comprise the carbon-subgroup surfactants and d-transition metals. In a second aspect of the invention combinations of germanium, copper and vanadium comprise the carbon-subgroup surfactants and d-transition metals.

Further aspects, benefits and features of the invention will become apparent from the ensuing detailed description of the invention. The best mode, which is contemplated in practicing the invention, together with the manner of using the invention, are disclosed, and the property, in which exclusive rights are claimed, is set forth in each of a series of numbered claims at the conclusion of the detailed description.

## BRIEF DESCRIPTION OF THE DRAWINGS

The invention will be better understood, and further objects characterizing features, details, and advantages thereof will appear more clearly with reference to the drawings illustrating a presently preferred specific embodiment of the invention by way of non-limiting example only.

The tables given below contain specific chemical compositions of steels belonging to different classes, as well as their mechanical and some operational properties after various types of heat treatment (quenching+tempering), carburizing and nitriding.

FIG. 1 is a table of universal steels according to the invention.

FIG. 2 is a table of a pair of high-ductility steels according to the invention.

FIG. 3 is a table of a pair of case hardening steels according to the invention.

FIG. 4 is a table of direct hardening, nitriding steel according to the invention.

FIG. 5 is a table of another direct hardening, nitriding steel according to the invention.

FIG. 6 is a table of a pair of direct hardening, nitriding steels and their operational properties according to the invention.

FIG. 7 is a table of a pair of direct hardening, nitriding steels according to the invention.

FIG. 8 is a table of a pair of tool steels according to the invention.

FIG. 9 is a table of a pair of corrosion-resistant, high-ductility steels according to the invention.

FIG. 10 is a table of a pair of corrosion-resistant, direct hardening steels according to the invention.

FIG. 11 is a table of a pair of corrosion-resistant direct hardening steels according to the invention, and their corrosion resistance in various aggressive environments.

FIG. 12 is a table of a pair of corrosion-resistant tool steels according to the invention.

FIG. 13 is a table of a pair of maraging steels according to the invention.

#### DETAILED DESCRIPTION OF THE PREFERRED EMBODIMENT

The present invention is a fundamentally new and universal alloying system and method for improving the mechanical properties of steel, reducing the classes and grades of specialty steels, reducing investment costs, reducing inventory costs, reducing steel-making operating costs, as well as the costs of machine-building facilities. The invention was developed after extensive studies of the effect various alloying elements have on the steel structure and properties, taking into account their electron structure, adsorption activity with respect to free metal surfaces, grain and phase boundaries, as well as changes in electron density of solid solutions of the substitutional elements (Al, Si, Cr, V, Ti, Nb, Zr, Mo, W, Co, Ni, Cu, Ge) and interstitial elements (C, N, O, H, S, P) in  $\alpha$ -iron and  $\gamma$ -iron.

The essence of the invention is that when certain combinations of small amounts of a complex of carbon-subgroup surfactants, such as silicon and germanium, and d-transition metals, such as copper and vanadium, are added to  $\alpha$  or ( $\alpha+\gamma$ ) iron-based alloys, containing 0.08 to 0.65 wt % of carbon; 0.35 to 0.75 wt % of manganese (with the exception of expansions shown below); and 0.60 to 18 wt % of chromium, the following benefits are obtained: 1. The diffusion of interstitial elements C, N, O, and H can be modified and controlled. 2. The formation or non-equilibrium segregations of the traditionally harmful admixtures of P, S, Sb, etc. and brittle phases on free metal surfaces, grain, and phase boundaries can be prevented or reduced. 3. The kinetics of phase transformations in steels during heating and cooling can be modified and controlled.

The relationship between the carbon-subgroup surfactants and the d-transition metals, which produce the above improvements, is as follows:

$$5 \quad (A+B)/C=k$$

where k stands for a constant, A stands for a carbon-subgroup surfactant, B stands for the d-transition metal copper, and C stands for the d-transition metal vanadium.

In a first embodiment of the invention, A stands for 0.75 to 1.50 wt % of silicon; B stands for 0.40 to 0.80 wt % of copper; and k is within the range of 2 to 14.

In a second embodiment of the invention, A stands for 0.60 to 1.50 wt % of germanium; B stands for 0.40 to 0.80 wt % of copper; and k is within the range of 4 to 11.

For each of the above embodiments, the different classes of universal alloy steels shown in FIG. 1 were developed and studied. The classes are expressed as the points carbon followed by the percentages of other elements. By way of example, the maraging steel in FIG. 1 is comprised of 0.10 percent carbon; 10 percent chromium, 8 percent nickel and the elements A, B, C, as disclosed in the above-described embodiments.

25 Except for the Ni of the 10Cr10Ni8ABC maraging steel, none of the above steels require the scarce and expensive alloying elements: Mo, Ni, W, Nb, N, B, Co. Moreover, with my invention, different specialty steels, including corrosion-resistant and maraging steels, can be produced by merely adding different amounts of carbon during a continuous casting of ingots and subsequent thermomechanical treatments while maintaining the same amounts of other elements. The following compositions are illustrative of the best mode, which is contemplated for practicing my 30 invention, reference being made to FIGS. 1 through 13, for 35 mechanical properties of specimens of said alloy steels:

| A. General Engineering Steel |                               |           |
|------------------------------|-------------------------------|-----------|
| I                            | High Ductility Steel (FIG. 2) |           |
|                              | [0040] a.                     |           |
|                              | Carbon                        | 0.08-0.18 |
|                              | Manganese                     | 0.35-0.75 |
|                              | Silicon                       | 0.75-1.50 |
|                              | Chromium                      | 0.60-3.00 |
|                              | Copper                        | 0.40-0.80 |
|                              | Vanadium                      | 0.10-0.35 |
|                              | Iron remainder                |           |
|                              | [0041] b.                     |           |
|                              | Carbon                        | 0.08-0.18 |
|                              | Manganese                     | 0.35-0.75 |
|                              | Silicon                       | 0.17-0.45 |
|                              | Chromium                      | 0.60-3.00 |
|                              | Germanium                     | 0.60-1.50 |
|                              | Copper                        | 0.40-0.80 |
|                              | Vanadium                      | 0.10-0.35 |
|                              | Iron remainder                |           |
| II                           | Case Hardening Steel (FIG. 3) |           |
|                              | [0042] b.                     |           |
|                              | Carbon                        | 0.08-0.28 |
|                              | Manganese                     | 0.17-0.81 |
|                              | Silicon                       | 0.75-1.50 |
|                              | Chromium                      | 0.60-3.00 |
|                              | Copper                        | 0.40-0.80 |
|                              | Vanadium                      | 0.10-0.35 |
|                              | Iron remainder                |           |
|                              | [0043] b.                     |           |
|                              | Carbon                        | 0.18-0.28 |
|                              | Manganese                     | 0.35-0.75 |
|                              | Silicon                       | 0.18-0.45 |
|                              | Chromium                      | 0.60-3.00 |
|                              | Germanium                     | 0.60-1.50 |
|                              | Copper                        | 0.40-0.80 |
|                              | Vanadium                      | 0.10-0.35 |
|                              | Iron remainder                |           |

-continued

-continued

|        |                               |                |            |   |        |        |                |                |                         |
|--------|-------------------------------|----------------|------------|---|--------|--------|----------------|----------------|-------------------------|
| [0044] | a.                            | Carbon         | 0.28–0.45  | 5 | [0054] | a.     | Carbon         | 0.28–0.56      |                         |
|        |                               | Manganese      | 0.27–0.75  |   |        |        | Manganese      | 0.27–0.75      |                         |
|        |                               | Silicon        | 0.75–1.50  |   |        |        | Silicon        | 0.75–1.50      |                         |
|        |                               | Chromium       | 0.60–3.00  |   |        |        | Chromium       | 12.5–18.00     |                         |
|        |                               | Copper         | 0.40–0.80  |   |        |        | Copper         | 0.40–0.80      |                         |
|        |                               | Vanadium       | 0.10–0.35  |   |        |        | Vanadium       | 0.10–0.35      |                         |
|        |                               | Iron remainder |            |   |        |        | Iron remainder |                |                         |
|        |                               | Carbon         | 0.28–0.45  |   | 10     | [0055] | b.             | Carbon         | 0.28–0.56               |
|        |                               | Manganese      | 0.35–0.75  |   |        |        |                | Manganese      | 0.24–0.75               |
|        |                               | Silicon        | 0.18–0.45  |   |        |        |                | Silicon        | 0.17–0.45               |
|        |                               | Chromium       | 0.60–3.00  |   |        |        |                | Chromium       | 12.5–18.00              |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
| [0045] | b.                            | Carbon         | 0.28–0.45  |   |        |        |                | Carbon         | 0.28–0.56               |
|        |                               | Manganese      | 0.35–0.75  |   |        |        |                | Manganese      | 0.24–0.75               |
|        |                               | Silicon        | 0.18–0.45  |   |        |        |                | Silicon        | 0.17–0.45               |
|        |                               | Chromium       | 0.60–3.00  |   |        |        |                | Chromium       | 12.5–18.00              |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.45–0.55  |   | 15     | [0056] | a.             | Carbon         | 0.56–0.65               |
|        |                               | Manganese      | 0.35–0.78  |   |        |        |                | Manganese      | 0.17–0.75 (per FIG. 12) |
|        |                               | Silicon        | 0.75–1.50  |   |        |        |                | Silicon        | 0.75–1.50               |
|        |                               | Chromium       | 0.60–3.00  |   |        |        |                | Chromium       | 12.5–18.00              |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
| [0046] | a.                            | Carbon         | 0.45–0.55  |   |        |        |                | Carbon         | 0.56–0.65               |
|        |                               | Manganese      | 0.35–0.78  |   |        |        |                | Manganese      | 0.17–0.75 (per FIG. 12) |
|        |                               | Silicon        | 0.75–1.50  |   |        |        |                | Silicon        | 0.75–1.50               |
|        |                               | Chromium       | 0.60–3.00  |   |        |        |                | Chromium       | 12.5–18.00              |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.45–0.55  |   |        |        |                | Carbon         | 0.56–0.65               |
|        |                               | Manganese      | 0.35–0.75  |   |        |        |                | Manganese      | 0.21–0.75               |
|        |                               | Silicon        | 0.18–0.45  |   |        |        |                | Silicon        | 0.18–0.45               |
| [0047] | b.                            | Chromium       | 0.60–3.00  |   |        |        |                | Chromium       | 12.5–18.00              |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.55–0.65  |   |        |        |                | Carbon         | 0.56–0.65               |
|        |                               | Manganese      | 0.35–0.81  |   |        |        |                | Manganese      | 0.21–0.75               |
|        |                               | Silicon        | 0.75–1.50  |   |        |        |                | Silicon        | 0.18–0.45               |
|        |                               | Chromium       | 0.60–3.00  |   |        |        |                | Chromium       | 12.5–18.00              |
|        |                               | Copper         | 0.40–0.80  |   |        |        |                | Copper         | 0.40–0.80               |
| [0048] | a.                            | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.55–0.65  |   |        |        |                | Carbon         | 0.56–0.65               |
|        |                               | Manganese      | 0.35–0.81  |   |        |        |                | Manganese      | 0.21–0.75               |
|        |                               | Silicon        | 0.75–1.50  |   |        |        |                | Silicon        | 0.18–0.45               |
|        |                               | Chromium       | 0.60–3.00  |   |        |        |                | Chromium       | 12.5–18.00              |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.55–0.65  |   |        |        |                | Carbon         | 0.56–0.65               |
| [0049] | b.                            | Manganese      | 0.35–0.75  |   |        |        |                | Manganese      | 0.21–0.75               |
|        |                               | Silicon        | 0.32–0.45  |   |        |        |                | Silicon        | 0.18–0.45               |
|        |                               | Chromium       | 0.60–3.00  |   |        |        |                | Chromium       | 12.5–18.00              |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.55–0.65  |   |        |        |                | Carbon         | 0.56–0.65               |
|        |                               | Manganese      | 0.35–0.75  |   |        |        |                | Manganese      | 0.21–0.75               |
|        |                               | Silicon        | 0.32–0.45  |   |        |        |                | Silicon        | 0.18–0.45               |
| VI     | Maraging Steel (FIG. 13)      | Chromium       | 9.50–12.50 |   |        |        |                | Chromium       | 9.50–12.50              |
|        |                               | Nickel         | 3.50–8.50  |   |        |        |                | Nickel         | 3.50–8.50               |
|        |                               | Silicon        | 0.75–1.50  |   |        |        |                | Silicon        | 0.75–1.50               |
|        |                               | Copper         | 0.40–0.80  |   |        |        |                | Copper         | 0.40–0.80               |
|        |                               | Vanadium       | 0.10–1.00  |   |        |        |                | Vanadium       | 0.10–1.00               |
|        |                               | Iron remainder |            |   |        |        |                | Iron remainder |                         |
|        |                               | Carbon         | 0.05–0.22  |   |        |        |                | Carbon         | 0.05–0.22               |
|        |                               | Chromium       | 9.50–12.50 |   |        |        |                | Chromium       | 9.50–12.50              |
|        |                               | Nickel         | 3.50–8.60  |   |        |        |                | Nickel         | 3.50–8.60               |
|        |                               | Germanium      | 0.60–1.50  |   |        |        |                | Germanium      | 0.60–1.50               |
| [0051] | b.                            | Copper         | 0.40–0.80  |   |        |        |                | Copper         | 0.40–0.80               |
|        |                               | Vanadium       | 0.10–1.00  |   |        |        |                | Vanadium       | 0.10–1.00               |
|        |                               | Iron remainder |            |   |        |        |                | Iron remainder |                         |
|        |                               | Carbon         | 0.05–0.22  |   |        |        |                | Carbon         | 0.05–0.22               |
|        |                               | Chromium       | 9.50–12.50 |   |        |        |                | Chromium       | 9.50–12.50              |
|        |                               | Nickel         | 3.50–8.60  |   |        |        |                | Nickel         | 3.50–8.60               |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–1.00  |   |        |        |                | Vanadium       | 0.10–1.00               |
|        |                               | Iron remainder |            |   |        |        |                | Iron remainder |                         |
| VII    | High Ductility Steel (FIG. 9) | Carbon         | 0.08–0.28  |   |        |        |                | Carbon         | 0.08–0.28               |
|        |                               | Manganese      | 0.18–0.75  |   |        |        |                | Manganese      | 0.18–0.75               |
|        |                               | Silicon        | 0.75–1.50  |   |        |        |                | Silicon        | 0.75–1.50               |
|        |                               | Chromium       | 12.5–18.00 |   |        |        |                | Chromium       | 12.5–18.00              |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.08–0.28  |   |        |        |                | Carbon         | 0.08–0.28               |
|        |                               | Manganese      | 0.21–0.75  |   |        |        |                | Manganese      | 0.21–0.75               |
|        |                               | Silicon        | 0.14–0.45  |   |        |        |                | Silicon        | 0.14–0.45               |
| [0053] | b.                            | Chromium       | 12.5–18.00 |   |        |        |                | Chromium       | 12.5–18.00              |
|        |                               | Germanium      | 0.60–1.50  |   |        |        |                | Germanium      | 0.60–1.50               |
|        |                               | Copper         | 0.40–0.80  |   |        |        |                | Copper         | 0.40–0.80               |
|        |                               | Vanadium       | 0.10–0.35  |   |        |        |                | Vanadium       | 0.10–0.35               |
|        |                               | Iron remainder |            |   |        |        |                | Iron remainder |                         |
|        |                               | Carbon         | 0.08–0.28  |   |        |        |                | Carbon         | 0.08–0.28               |
|        |                               | Manganese      | 0.21–0.75  |   |        |        |                | Manganese      | 0.21–0.75               |
|        |                               | Silicon        | 0.14–0.45  |   |        |        |                | Silicon        | 0.14–0.45               |
|        |                               | Chromium       | 12.5–18.00 |   |        |        |                | Chromium       | 12.5–18.00              |
|        |                               | Germanium      | 0.60–1.50  |   |        |        |                | Germanium      | 0.60–1.50               |

\* \* \* \* \*

30 From the foregoing, it will be understood that my universal alloy steel is a fundamentally new composition and method, which provide substantial benefits over current practices. In addition to improving the mechanical properties of steel, it reduces complexity and the costs of establishing and maintaining large inventories and facilities.

40 Although only several embodiments of my invention have been described, it will be appreciated that other embodiments can be developed by changes, such as substitution and addition of elements, and changes in the amounts of an element, without departing from the spirit thereof.

45 What is claimed is:

1. An alloy steel composition produced by conventional means and characterized by a combination of high strength, ductility and toughness, the composition consisting by weight percent essentially of: from more than 0.45 to 0.65 of carbon; about 0.75–1.50 of silicon; from more than 0.40 to less than 0.65 of copper; about 0.10–0.35 of vanadium; and about 0.60–3.00 of chromium, the remainder being iron, manganese and incidental impurities.

50 2. An alloy steel composition with superior impact strength, particularly at low temperatures, consisting by weight percent essentially of: from more than 0.45 to 0.55 of carbon; about 0.75–1.5 of silicon; about 0.35–0.75 of manganese; about 0.40–0.80 of copper; about 0.10–0.35 of vanadium; about 0.6–1.6 of chromium, the remainder being iron and incidental impurities.

55 3. An alloy steel composition for manufacturing tools and dies with superior toughness and impact strength, particularly at low temperatures, consisting by weight percent essentially of: about 0.55–0.65 of carbon; about 0.75–1.5 of silicon; about 0.40–0.80 of copper; about 0.10–0.35 of vanadium; and about 0.60–3.0 of chromium; the remainder being iron, manganese, and incidental impurities.